

## UNITED STATES PATENT OFFICE

2,173,029

## PROCESS FOR RENDERING TEXTILES WATER-REPELLENT AND PRODUCTS THEREFROM

Ernst Waltmann and Edgar Wolf, Krefeld, Germany, assignors to Heberlein Patent Corporation, New York, N. Y., a corporation of New York

No Drawing. Application February 18, 1937, Serial No. 1,26,521. In Germany February 19, 1936

6 Claims. (Cl. 8—120)

This invention relates to processes for producing water-repellent fibrous materials and products therefrom.

In our copending application Serial No. 76,738, filed April 28, 1936, there is described a process for treating material with an isocyanate to increase the water-repellence thereof and the product obtained therefrom. We have now found that isocyanates of another formula may be employed for the production of water-repellent fibrous materials, and have also found novel processes for producing the substances employed for rendering the materials water-repellent.

The principal object of the present invention is to provide a simple process to increase water-repellence in materials such as cotton, jute, linen, hemp and various artificial silks and wool, presenting advantages over the known fatty acid chloride and fatty acid anhydride processes referred to in said copending application.

The invention accordingly comprises the novel products as well as the novel processes and steps of processes according to which such products are manufactured, the specific embodiments of which are described hereinafter by way of example and in accordance with which we now prefer to practice the invention.

We have found in accordance with our invention that isocyanate derivatives having the general formula  $R.CO.N=C=O$  can be employed with great success for rendering textiles water-repellent. In the formula just mentioned and in the appended claims in which said formula is employed,  $R$  is intended to designate an alkyl, cycloalkyl or aralkyl radical containing a saturated alkyl radical of at least 10 carbon atoms or signifies the saturated or unsaturated radical of an alcohol of the sterol series. Textile materials such as cotton, jute, linen, hemp and various artificial silks and wool may be treated with such materials to produce a slight surface combination to produce the desired water-repellence. In the case of cellulose it is believed that there is a reaction with the cellulose molecule by the herein described isocyanates to produce a carbamic acid ester of the cellulose. In the case of the cellulose derivatives a similar reaction occurs and in the case of wool the reaction with the isocyanate is believed to produce substituted urea derivatives. The result of this action is to produce a surface structure which is water-repellent.

Materials falling under the formula mentioned above are distinguished by extremely high rapidity of reaction toward textile materials, particularly towards cellulose and cellulose deriva-

tives. It is necessary only to bring the textile material in contact with the isocyanate as by passing the textile material briefly through a solution of the substance in benzine or a suitable solvent and immediately thereafter subjecting it for several minutes to a high temperature, usually 100° C. or above.

Impregnation of the textile materials with the esters herein mentioned may be carried out in any desired manner with or without the use of organic solvents by means of emulsification in an aqueous solution by soaking, spraying or the like. It is also possible in the case of acetyl cellulose to add the isocyanates mentioned herein to the spinning solution itself in order thus to combine the process of producing water-repellence with the spinning process. Also one may treat the fibers of cellulose or cellulose derivatives immediately after the spinning process with the esters herein mentioned to obtain water-repellence. The addition of catalytic agents, such as pyridine for the purpose of securing the desired effect, may be made but such addition is not necessary. The water-repellent effect secured by these treatments resists domestic washing. After thorough rinsing out with soap employed in such washing and drying, the textile material again manifests water-repellent properties. It is also resistant to dry cleaning.

The substances falling under the above formula may be obtained by the action of isocyanates upon acid chlorides (cf. Ber. 36, page 3213, C. Billeter). The reaction proceeds according to the following formula:



These substances may also be prepared by causing fatty acid amides to react with phosgene to produce acyl carbamic acid chlorides. Upon treatment of these materials with calcium oxide or similar oxide, the corresponding acid isocyanate is obtained. The reactions are as follows:



According to a modification of the process the said higher acyl-isocyanates may be replaced by the corresponding acyl-carbamic-acid chlorides. These compounds may be obtained by treating fatty acid amides with phosgene (cf. German Patent No. 566,603).

Employing higher acyl-carbamic acid chlorides

instead of the corresponding acyl-isocyanates the textile materials are advantageously treated before impregnation takes place with weak aqueous solutions of sodium hydroxide, sodium carbonate or sodium acetate.

Also in a modification organic bases such as pyridine may be added to the solutions of acyl carbamic chlorides in organic solvents.

The following examples represent preferred embodiments of the invention for producing water-repellence in accordance with the manner in which we now prefer to practice it. It is to be understood that these examples are illustrative and the invention is not to be considered as limited thereto except as indicated in the appended claims.

#### Examples

(1) A raincoat material, having spun viscose rayon as warp and weft, is passed through a 1% solution of stearic acid isocyanate



in benzol for 3 seconds at a temperature of 25° C., and after evaporating of the benzol is heated for 5 minutes to 140° C. (284° F.). The material then becomes water-repellent. The effect is proof to washing with soap, as well as to the solvents customary in dry cleaning.

(2) A cellulose hydrate web is passed through a 1% solution of palmitic acid isocyanate



in benzol for 4 seconds at a temperature of 25° C. and after evaporating of the benzol is heated for 60 minutes to 120° C. (248° F.). The resulting effect is similar to that of Example 1.

(3) A wool muslin is passed through a 1% solution of stearic acid-isocyanate in carbon tetrachloride for 3 seconds at a temperature of 25° C. and after evaporating of the solvent is heated for 60 minutes to 120° C. (248° F.). The result is similar to that of Example 1.

(4) A poplin from mercerized cotton is passed through 1% solution of stearic acid-butyl-carbamic acid chloride in benzol for 4 seconds at a temperature of 25° C. The solution also contains 10 grams of pyridine per liter. After evaporating of the benzol the material is heated for 60 minutes to 60° C. (140° F.). The resulting effect is similar to that of Example 1.

(5) A cotton tent cloth is passed through an aqueous solution of 10 grams per liter of sodium acetate, dried, and then passed through a 1% solution of palmitic acid methyl carbamic acid chloride



in carbon tetrachloride for 4 seconds at a temperature of 25° C. After evaporating of the solvent the material is heated 60 minutes to 70° C. (158° F.). The resulting effect is similar to that of Example 1.

(6) A clothing material of cuprammonium silk is passed through a 1% solution of phenyl-stearic acid isocyanate in benzol for 3 seconds at a temperature of 25° C., and after evaporating of the benzol is heated for 5 minutes to 140° C. (284° F.). The material then becomes water-repellent. The effect is proof to washing with soap, as well as to the solvents customary in dry cleaning (manufacture of phenyl-stearic acid c. f. United States Patent No. 1,972,568).

For the production of the substances for pro-

ducing water-repellence, the following are examples of the way in which we now prefer to practice the invention. The invention is not to be restricted thereto, however, except as indicated in the appended claims.

(7) A mixture of 284 parts by weight of stearic acid chloride and 150 parts by weight of silver cyanate are heated in 300 parts by weight of toluene at the reflux condenser for 60 minutes. The solution of stearic acid isocyanate  $C_{17}H_{35}CO.N=C=O$  is liberated from the precipitated chloride by filtration.

(8) A mixture of 256 parts by weight of palmitic acid chloride and 82 parts by weight of potassium cyanate dissolved in a small quantity of water are heated in 300 parts by weight of toluene at the reflux condenser for 30 minutes. Palmitic acid isocyanate  $C_{15}H_{31}CO.N=C=O$  is liberated from the precipitated potassium chloride by filtration.

There are suitable also the acyl-isocyanates which are obtained by transposition of higher fatty acid amides with phosgene. This transposition is effected as follows:

(9) 250 parts by weight of stearic acid amide are dissolved in 700 parts by weight of toluene 80 parts by weight of pyridine and 100 parts by weight of phosgene are added. The mixture is heated in an autoclave to 150° C. for three hours. Stearic acid-carbamic acid chloride is obtained. The corresponding isocyanate is obtained by dissolving the acyl-carbamic acid chloride in benzene and heating it with calcium oxide.

(10) Carbamic acid chlorides may be made as follows: 300 parts by weight of stearic acid butyl-amide are dissolved in 700 parts by weight of toluene, 80 parts by weight of pyridine and 100 parts by weight of phosgene are added. The mixture is heated in an autoclave to 150° C. for a few hours. Stearic acid-butyl-carbamic acid chloride



is obtained.

(11) 250 parts by weight of palmitic acid methylamide are dissolved in 700 parts by weight of toluene, 80 parts by weight of pyridine and 100 parts by weight of phosgene are added. The mixture is heated in an autoclave to 150° C. for a few hours. Palmitic acid methyl carbamic acid chloride



is obtained.

The amount of the ester deposited in all of the above examples on the textile materials will naturally vary with the weight of the material and its reactivity. We have found that ordinarily an amount of the ester equal to about 1% of the material is sufficient to give the effect. Corresponding amounts of the chlorides are also deposited.

The materials produced in accordance with the above examples show a high degree of water-repellence. They show a lesser absorption of moisture as compared with the known processes for treatment with fatty acid chlorides and fatty acid anhydrides. They show also greatly improved durability toward dry-cleaning, soap washing, etc. as compared with these previous materials. The feel and hang of the materials having water-repellence as produced above, have not been substantially altered.

The process of the invention, particularly as set forth in the specific embodiments above, may be carried out with simple apparatus at relatively small expense and in a relatively short time.

5 In the claims where the expression "textile material" is employed, it is intended to cover fibers, yarns, fabrics or other forms of wool or cellulose-containing materials including cotton, jute, linen, hemp or rayon including viscose, cuprammonium, or other precipitated cellulose or derivatives of cellulose such as acetyl cellulose.

10 While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes 15 and modifications.

20 Subject matter not claimed herein is claimed in our copending applications: Serial No. 76,738, filed April 28, 1936; Serial No. 289,394, filed August 10, 1939; Serial No. 289,395, filed August 10, 25 1939; and Serial No. 289,396, filed August 10, 1939.

25 What is claimed as new and desired to be secured by Letters Patent, is:

1. A process for ennobling textile material which comprises impregnating the material with 30 an isocyanic acid ester having the formula R.CO.N=C=O in which formula R signifies an alkyl, cycloalkyl or aralkyl radical containing a saturated alkyl radical of at least 10 carbon atoms or signifies a saturated or unsaturated 35 radical of an alcohol of the sterol series and heating the impregnated material to increase the water-repellence thereof.

2. A process for ennobling textile material which comprises impregnating the material with 40 an isocyanic acid ester of an organic acid having a saturated alkyl radical of at least 10 carbon

atoms in which the isocyanate group N=C=O is directly linked to the carbonyl group CO and heating the impregnated material to increase the water-repellence thereof.

3. A process for ennobling textile material 5 which comprises impregnating the material with an isocyanic acid ester of an organic acid containing a sterol group in which the isocyanate group N=C=O is linked directly with the carbonyl group CO, and heating the impregnated 10 material to increase the water-repellence.

4. A process for ennobling textile material 15 which comprises subjecting the material to reaction with stearyl isocyanate at a temperature of about 150° C. for about 5 minutes to increase the water-repellence of said material.

5. A textile material partially chemically altered with an isocyanate of the formula 20 R.CO.N=C=O and in which formula R signifies an alkyl, cycloalkyl or aralkyl radical containing a saturated alkyl radical of at least 10 carbon atoms or signifies the saturated or unsaturated 25 radical of an alcohol of the sterol series, said material having a water-repellent property but in appearance and feel being substantially the same as similar material untreated, said material being also capable of withstanding ordinary house laundering and other cleaning.

6. A textile material treated with an isocyanic 30 acid ester of an organic acid having a saturated alkyl radical of at least 10 carbon atoms in which the isocyanate group N=C=O is directly linked to the carbonyl group CO, to produce in said material, a water-repellent property, said material in appearance and feel being substantially 35 the same as similar material untreated, said material being also capable of withstanding ordinary house laundering and dry cleaning.

ERNST WALTSMANN. 40  
EDGAR WOLF.

CERTIFICATE OF CORRECTION.

Patent No. 2,173,029.

September 12, 1939.

ERNST WALTSMANN, ET AL.

It is hereby certified that error appears in the printed specification of the above numbered patent requiring correction as follows: Page 2, second column, lines 34 and 35, strike out the words and colon "Carbamic acid chlorides may be made as follows:" and insert the same as a separate paragraph after "oxide.", line 33, Example 9; and that the said Letters Patent should be read with this correction therein that the same may conform to the record of the case in the Patent Office.

Signed and sealed this 3rd day of October, A. D. 1939.

(Seal)

Henry Van Arsdale,  
Acting Commissioner of Patents.

The process of the invention, particularly as set forth in the specific embodiments above, may be carried out with simple apparatus at relatively small expense and in a relatively short time.

5 In the claims where the expression "textile material" is employed, it is intended to cover fibers, yarns, fabrics or other forms of wool or cellulose-containing materials including cotton, jute, linen, hemp or rayon including viscose, cuprammonium, or other precipitated cellulose or derivatives of cellulose such as acetyl cellulose.

10 While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes 15 and modifications.

20 Subject matter not claimed herein is claimed in our copending applications: Serial No. 76,738, filed April 28, 1936; Serial No. 289,394, filed August 10, 1939; Serial No. 289,395, filed August 10, 25 1939; and Serial No. 289,396, filed August 10, 1939.

25 What is claimed as new and desired to be secured by Letters Patent, is:

1. A process for ennobling textile material which comprises impregnating the material with 30 an isocyanic acid ester having the formula R.CO.N=C=O in which formula R signifies an alkyl, cycloalkyl or aralkyl radical containing a saturated alkyl radical of at least 10 carbon atoms or signifies a saturated or unsaturated 35 radical of an alcohol of the sterol series and heating the impregnated material to increase the water-repellence thereof.

2. A process for ennobling textile material which comprises impregnating the material with 40 an isocyanic acid ester of an organic acid having a saturated alkyl radical of at least 10 carbon

atoms in which the isocyanate group N=C=O is directly linked to the carbonyl group CO and heating the impregnated material to increase the water-repellence thereof.

3. A process for ennobling textile material 5 which comprises impregnating the material with an isocyanic acid ester of an organic acid containing a sterol group in which the isocyanate group N=C=O is linked directly with the carbonyl group CO, and heating the impregnated 10 material to increase the water-repellence.

4. A process for ennobling textile material 15 which comprises subjecting the material to reaction with stearyl isocyanate at a temperature of about 150° C. for about 5 minutes to increase the water-repellence of said material.

5. A textile material partially chemically altered with an isocyanate of the formula 20 R.CO.N=C=O and in which formula R signifies an alkyl, cycloalkyl or aralkyl radical containing a saturated alkyl radical of at least 10 carbon atoms or signifies the saturated or unsaturated 25 radical of an alcohol of the sterol series, said material having a water-repellent property but in appearance and feel being substantially the same as similar material untreated, said material being also capable of withstanding ordinary house laundering and other cleaning.

6. A textile material treated with an isocyanic 30 acid ester of an organic acid having a saturated alkyl radical of at least 10 carbon atoms in which the isocyanate group N=C=O is directly linked to the carbonyl group CO, to produce in said material, a water-repellent property, said material in appearance and feel being substantially 35 the same as similar material untreated, said material being also capable of withstanding ordinary house laundering and dry cleaning.

ERNST WALTSMANN. 40  
EDGAR WOLF.

CERTIFICATE OF CORRECTION.

Patent No. 2,173,029.

September 12, 1939.

ERNST WALTSMANN, ET AL.

It is hereby certified that error appears in the printed specification of the above numbered patent requiring correction as follows: Page 2, second column, lines 34 and 35, strike out the words and colon "Carbamic acid chlorides may be made as follows:" and insert the same as a separate paragraph after "oxide.", line 33, Example 9; and that the said Letters Patent should be read with this correction therein that the same may conform to the record of the case in the Patent Office.

Signed and sealed this 3rd day of October, A. D. 1939.

(Seal)

Henry Van Arsdale,  
Acting Commissioner of Patents.